

**United States Patent** [19]**Buchanan et al.****[11] Patent Number:** **5,019,492****[45] Date of Patent:** **May 28, 1991**

[54] **PHOTOGRAPHIC ELEMENT AND  
PROCESS COMPRISING A BLOCKED  
PHOTOGRAPHICALLY USEFUL  
COMPOUND**

[75] Inventors: **John M. Buchanan; Ewell R. Cook;  
Jared B. Mooberry; Gary S. Proehl,  
all of Rochester; Stephen P. Singer,  
Spencerport, all of N.Y.; William N.  
Washburn, LaJolla, Calif.**

[73] Assignee: **Eastman Kodak Company,  
Rochester, N.Y.**

[21] Appl. No.: **343,981**

[22] Filed: **Apr. 26, 1989**

[51] Int. Cl.<sup>5</sup> ..... **G03C 7/305**

[52] U.S. Cl. ..... **430/543, 430/218;  
430/219; 430/222; 430/223; 430/544; 430/559;  
430/607; 430/610; 430/611; 430/598; 430/621;  
430/955; 430/956; 430/957; 430/958; 430/959;  
430/960**

[58] **Field of Search** ..... **430/955, 956, 957, 958,  
430/959, 960, 598, 543, 544, 559, 607, 610, 611,  
218, 219, 222, 223; 436/621**

[56] **References Cited**

**U.S. PATENT DOCUMENTS**

4,248,962 3/1981 Lau ..... 430/382  
4,263,393 4/1981 Chen ..... 430/218  
4,283,472 8/1981 Gompf et al. ..... 430/17  
4,310,612 1/1982 Mooberry et al. ..... 430/223  
4,358,525 11/1982 Mooberry et al. ..... 430/217

4,409,323 10/1983 Sato et al. ..... 430/544  
4,446,216 5/1984 Smith et al. ..... 430/405  
4,554,243 11/1985 Ono et al. ..... 430/543  
4,629,683 12/1986 Itoh et al. ..... 430/390  
4,690,885 9/1987 Yagihara ..... 430/219  
4,737,442 4/1988 Yagihara et al. ..... 430/264  
4,772,537 9/1988 Itoh et al. ..... 430/219  
4,857,440 8/1989 Begley et al. ..... 430/382

**FOREIGN PATENT DOCUMENTS**

0255085 2/1988 European Pat. Off. .

*Primary Examiner*—Charles L. Bowers, Jr.

*Assistant Examiner*—Lee C. Wright

*Attorney, Agent, or Firm*—Richard E. Knapp

[57]

**ABSTRACT**

A novel blocked photographically useful compound comprises a new blocking group that (a) comprises two electrophilic groups, the least electrophilic of which is bonded directly or through a timing group to the photographically useful group (PUG) of the compound, (b) is capable of reacting with a dinucleophile reagent, and (c) has the two electrophilic groups separated from each other by a bond or unsubstituted or substituted atom that enables nucleophilic displacement to occur with release of PUG when the compound is reacted with a dinucleophile reagent. Such a blocked photographically useful compound is useful in a photographic material and process to provide increased stability and enable more rapid release of the photographically useful group upon reaction with a dinucleophile reagent.

**8 Claims, No Drawings**

**PHOTOGRAPHIC ELEMENT AND PROCESS  
COMPRISING A BLOCKED  
PHOTOGRAPHICALLY USEFUL COMPOUND**

This invention relates to a new blocked photographically useful compound that is capable of more rapidly releasing the photographically useful group of the compound upon reaction of the compound with a dinucleophile reagent.

Various compounds, such as couplers and dyes, are known in the photographic art that contain a blocking group and that are capable of being released or unblocked upon processing of the photographic material containing the compound. Such compounds and various blocking groups have been described in, for example, U.S. Pat. Nos. 4,690,885; 4,358,525 and 4,554,243. While these compounds have enabled increased storage stability compared to compounds that are not blocked and have provided release of the photographically useful group from the compound upon processing, often the stability of the compounds during storage prior to exposure and processing of the photographic materials containing the compounds has not been entirely satisfactory and the rate of release or unblocking of the compound has been less than desired.

A need has existed for a blocked photographically useful compound containing a blocking group that enables increased storage stability in a photographic material and enables increased rate of release or unblocking during processing of the photographic material without adverse effects upon a photographic material containing such a compound.

The present invention solves these problems by providing a photographic element comprising a support bearing at least one photographic silver halide emulsion layer and a blocked photographically useful compound comprising a photographically useful group (PUG) and a new blocking group that is capable of releasing the PUG upon processing the photographic element wherein the blocking group (a) comprises two electrophilic groups, the least electrophilic of which is bonded directly or through a timing group to the photographically useful group (PUG); (b) is capable of reacting with a dinucleophile; and, (c) the two electrophilic groups are separated from each other by a bond or unsubstituted or substituted atom that enables a nucleophilic displacement reaction to occur with release of PUG upon processing the photographic element in the presence of a dinucleophile reagent.

A preferred blocked photographically useful compound as described is represented by the formula:



wherein

$E_1$  and  $E_2$  are independently electrophilic groups, wherein  $E_1$  is more electrophilic than  $E_2$ ;  
 $T_1$  and  $T_2$  are individually releasable timing groups;  
 $Y^1$  is unsubstituted or substituted atom, preferably a carbon or nitrogen atom, that provides a distance between  $E_1$  and  $E_2$  that enables a nucleophilic displacement reaction to occur with release of PUG upon processing a photographic element containing the blocked photographically useful compound in the presence of a dinucleophile;

**2**  
PUG is a photographically useful group capable of being released upon processing the photographically useful compound;  
 $w$ ,  $x$  and  $y$  are independently 0 or 1; and,  
 $n$  is 1 or 2.

An illustrative blocked photographically useful compound within the above formula is represented by the formula:



15  
wherein  
 $\text{R}_3$  is unsubstituted or substituted alkyl, unsubstituted or substituted aryl, or the atoms necessary with  $Z$  to complete a ring, particularly an alicyclic or heterocyclic ring, with  $\text{Y}^2$ ;

20  
 $Z$  represents the atoms necessary to complete a ring with  $\text{R}_3$  and  $\text{Y}^2$

25  
 $\text{Y}^2$  is a substituted or unsubstituted carbon or nitrogen atom that provides a distance between the carbonyl groups that enables a nucleophilic displacement reaction to occur upon processing a photographic element containing the blocked photographically useful compound in the presence of a dinucleophile;  
 $q$  and  $z$  are independently 0 or 1;

30  
 $\text{T}_3$  is a releasable timing group; and,  
PUG is a photographically useful group.

Highly preferred blocked photographically useful compounds are represented by the formulas:



and



45  
50  
wherein  $\text{R}_{4a}$ ,  $\text{R}_{4b}$  and  $\text{R}_{4c}$  individually are unsubstituted or substituted alkyl or unsubstituted or substituted aryl; PUG is a photographically useful group;  $\text{T}_4$  and  $\text{T}_5$  are individually releasable timing groups; and  $r$  and  $s$  individually are 0 or 1.  $\text{R}_{4a}$ ,  $\text{R}_{4b}$  and  $\text{R}_{4c}$  are preferably methyl.

55  
55  
The blocking group as described can contain a ballast group. Ballast groups known in the photographic art can be used for this purpose.

One embodiment of the invention is a photographic element comprising a blocked photographically useful compound containing the new blocking group as described. Another embodiment is a process of forming a photographic image by developing an exposed photographic element as described in the presence of a dinucleophile reagent. A further embodiment is a new photographically useful compound containing the new blocking group as described.

The blocked photographically useful compounds enable both improved storage stability and more rapid

release upon processing of a photographic element containing such a compound. Both of these properties are achieved by the blocked photographically useful compounds as described due at least in part to the particular structure of the new blocking group. In the past it was possible for blocked photographically useful compounds to react with nucleophilic compounds containing one nucleophilic group, such as methylamine, hydroxide or water, that help reduce storage stability of the photographic element containing such compounds. The blocked photographically useful compounds of the invention do not release the photographically useful groups of the compound upon reaction with a nucleophilic compound containing only one nucleophilic group. Rather, release occurs only upon reaction with a nucleophilic compound containing two nucleophile groups, described herein as a dinucleophile reagent, such as hydroxylamines, hydrogen peroxide, hydrazine, diamines and substituted hydrazines. Carbonyl groups are preferred electrophilic groups in the new blocking groups as described.

The new blocking group structure resists reaction with nucleophilic compounds containing only one nucleophilic group. For example, reaction of a nucleophilic compound containing only one nucleophilic group at E<sub>1</sub> in the case of a carbonyl group would lead to adducts in which the hydroxyl group generated can internally react with E<sub>2</sub> only by a three or four member ring that is very difficult to form. In most cases, only compounds, such as water, that contain one nucleophilic group are encountered in storage of photographic silver halide elements. Such compounds would not release the blocking group of the invention as described.

In chemical systems requiring the good storage properties and the more rapid release properties of the compounds as described, the release of the blocking group can be initiated by reaction of the blocking group with an appropriate dinucleophile reagent. The selection of an appropriate dinucleophile reagent preferably enables formation of a five- or six-member ring compound. Depending upon the particular photographically useful group, the particular blocking group and the desired end use of the compound, the initiation of deblocking can take place by reacting the particular dinucleophile reagent at concentrations and under conditions that enable the desired rate of release.

The dinucleophile herein means a compound represented by the formula:



wherein Nu<sub>1</sub> and Nu<sub>2</sub> individually are nucleophilic N, O, S, P, Se, substituted nitrogen atoms, or substituted carbon atoms; X<sup>1</sup> is a chain of j atoms wherein j is 0, 1 or 2. Illustrative examples of useful dinucleophile reagents are as follows:

| j = 0                               | j = 1                                    | j = 2                                                                                                                    |
|-------------------------------------|------------------------------------------|--------------------------------------------------------------------------------------------------------------------------|
| H <sub>2</sub> O <sub>2</sub>       | NH <sub>2</sub> CONH <sub>2</sub>        | NH <sub>2</sub> CH <sub>2</sub> CH <sub>2</sub> NH <sub>2</sub>                                                          |
| NH <sub>2</sub> NH <sub>2</sub>     |                                          |                                                                                                                          |
| CH <sub>3</sub> NHNHCH <sub>3</sub> | NH <sub>2</sub> -C=NH<br>NH <sub>2</sub> | NH <sub>2</sub> CH <sub>2</sub> CO <sub>2</sub> H<br>NH <sub>2</sub> C(CH <sub>3</sub> ) <sub>2</sub> CH <sub>2</sub> OH |

-continued

| j = 0                                             | j = 1                                    | j = 2                                              |
|---------------------------------------------------|------------------------------------------|----------------------------------------------------|
| NH <sub>2</sub> OH                                |                                          | NH                                                 |
| CH <sub>3</sub> NHOH                              | CH <sub>3</sub> -C=NH<br>NH <sub>2</sub> | NH <sub>2</sub> CH <sub>2</sub> CH <sub>2</sub> SH |
| CH <sub>3</sub> C-NHOH                            |                                          |                                                    |
| CH <sub>3</sub> SO <sub>2</sub> NHNH <sub>2</sub> |                                          |                                                    |



Preferred dinucleophile reagents are hydroxylamine, hydrogen peroxide, and monosubstituted hydroxylamine. The dinucleophile reagent herein also includes a salt form of the reagent, such as the acid salts, for example, sulfate or bisulfite salts.

As used herein the term photographically useful group (PUG) refers to any group that can be used in a photographic material and that can be released from the blocking group as described. It refers to the part of the blocked photographically useful compound other than the blocking group. The PUG can be, for example, a photographic dye or photographic reagent. A photographic reagent herein is a moiety that upon release further reacts with components in the photographic element. Such useful photographically useful groups include, for example, couplers (such as, image dye-forming couplers, development inhibitor releasing couplers, competing couplers, polymeric couplers and other forms of couplers), development inhibitors, bleach accelerators, bleach inhibitors, inhibitor releasing developers, dye precursors, developing agents (such as competing developing agents, dye-forming developing agents, developing agent precursors, and silver halide developing agents), silver ion fixing agents, silver halide solvents, silver halide complexing agents, image toners, pre-processing and post-processing image stabilizers, hardeners, tanning agents, fogging agents, antifoggants, ultraviolet radiation absorbers, nucleators, chemical and spectral sensitizers or desensitizers, surfactants, and precursors thereof and other addenda known to be useful in photographic materials.

The PUG can be present in the photographically useful compound as a preformed species or as a precursor. For example, a preformed development inhibitor may be bonded to the blocking group or the development inhibitor may be attached to a timing group that is released at a particular time and location in the photographic material. The PUG may be, for example, a preformed dye or a compound that forms a dye after release from the blocking group.

The photographically useful compound can optionally contain at least one releasable timing group (T) between PUG and the blocking group as described. The reaction of the photographically useful compound with a dinucleophile reagent can sequentially release the blocking group from the timing group and then the timing group can be released from the PUG. The term "timing group" herein also includes a linking group that involves little or no observable time in the release action. This can occur in, for example, the development step of an exposed photographic element when the developer composition comprises a dinucleophile reagent, such as a hydroxylamine. Any timing group that is

known in the photographic art is useful as the timing group between PUG and the blocking group. Examples of useful timing groups are described in, for example, U.S. Pat. Nos. 4,248,962 and 4,409,323 and European Patent Application No. 255,085.

The particular timing groups employed, including the linkage by which they are attached to the PUG and the blocking group and the nature of the substituents on the timing group can be varied to help control such parameters as rate and time of bond cleavage of the blocking group and the PUG as well as diffusibility of the PUG and substituent groups.

If the PUG is joined to the blocking group only through the timing group, then the cleavage of the bond 15 between the timing group and the blocking group releases the timing group and the PUG as a unit. The particular timing group in this case can control the rate and distance of diffusion in the photographic material 20 before the PUG is released from the timing group. The timing group should not contain a structure that inhibits the reaction of the blocking group with a dinucleophile reagent.

In the formula as described timing groups  $T_1$  and  $T_2$  25 are independently selected to provide the desired rate and time of release of the PUG upon processing. The timing groups  $T_1$  and  $T_2$  can be the same or different. Examples of preferred timing groups for  $T_1$  and  $T_2$  are 30 as follows:



wherein  $E_2$  and PUG are as described; and,  $R_{4d}$ ,  $R_{4e}$ , and  $R_{4f}$  are hydrogen or substituents, such as alkyl, aryl, nitro, chloro and sulfonamido.

Other examples of useful timing groups are described in, for example, U.S. Pat. Nos. 4,248,962 and 4,772,537.

In the blocking group as described the two electrophilic groups,  $E_1$  and  $E_2$ , can be any electrophilic group that enables nucleophilic displacement reaction to occur upon reaction of the blocking group with a dinucleophile reagent. While carbonyl groups are highly preferred as the electrophilic groups, other examples of useful electrophilic groups are as follows:



wherein  $R_f$  is a substituent that causes the attached carbon atom to be an electrophilic center.

Highly preferred groups in the blocking group described containing  $Z$ ,  $Y^2$  and  $R_3$  are as follows:



wherein  $R_q$  is alkyl, such as methyl, ethyl, n-propyl, i-propyl, and butyl, or aryl, such as phenyl, benzyl or substituted phenyl or other substituents such as alkoxy, chloro and amido; and,



wherein  $R_4$  is as described;  $R_{4a}$  and  $R_{4b}$  are individually as described, such as methyl, ethyl, n-propyl, i-propyl, butyl, phenyl, benzyl, and substituted phenyl, or other substituents such as alkoxy, chloro and amido.

Illustrative examples of useful PUG's that can be blocked with the blocking groups as described are as follows:

## I. COUPLERS

A. Image Dye-Forming Couplers Illustrative couplers include cyan, magenta and yellow image dye-forming couplers that are known in the photographic art. Illustrative cyan dye-forming couplers that can comprise the blocking group, as described include, for example, those described in U.S. Pat. Nos. 2,772,162; 2,895,826; 3,002,836; 3,034,892; 2,474,293; 2,423,730;

2,367,531; 4,333,999; and 3,041,236. Illustrative magenta dye-forming couplers that can comprise the blocking group, as described include those described in, for example, U.S. Pat. Nos. 2,600,788; 2,369,489; 2,343,703; 2,311,082; 3,152,896; 3,152,896; 3,519,429; 3,062,653; and 2,908,573. Illustrative yellow dye-forming couplers that can contain the blocking group, as described include those described in, for example, U.S. Pat. Nos. 2,875,057; 2,407,210; 3,265,506; 2,298,443; 3,048,194; 10 and 3,447,928.

B. Illustrative couplers that form colorless products upon reaction with oxidized color developing agents and contain the blocking group, as described include those described in, for example, U.S. Pat. Nos. 15 3,632,345; 3,928,041; 3,958,993; 3,961,959; and U.K. Patent No. 861,138.

C. Illustrative couplers that form black dyes upon reaction with oxidized color developing agents and that can contain the blocking group, as described, include those described in, for example, U.S. Pat. Nos. 1,939,231; 2,181,944; 2,333,106; and 4,126,461; German OLS Nos. 2,644,194 and 2,650,764. 20

D. Illustrative couplers that are development inhibitor releasing couplers (DIR couplers) and can contain the blocking group, as described, include those described in, for example, U.S. Pat. Nos. 4,248,962; 3,227,554; 3,384,657; 3,615,506; 3,617,291; 3,733,201; and U.K. No. 1,450,479. Preferred development inhibitors as PUG's are heterocyclic compounds, such as mercaptotetrazoles, mercaptotriazoles, mercaptooxadiazoles, selenotetrazoles, mercaptobenzothiazoles, selenobenzothiazoles, mercaptobenzoxazoles, selenobenzoxazoles, mercaptobenzimidazoles, selenobenzimidazoles, benzotriazoles, benzodiazoles and 1,2,4-triazoles, tetrazoles, and imidazoles.

E. PUG's that are, or form, dyes upon release: Useful dyes and dye precursors include azo, azomethine, 40 azopyrazolone, indoaniline, indophenol, anthraquinone, triaryl methane, alizarin, nitro, quinoline, indigoid, oxanol, and phthalocyanine dyes and precursors of such dyes, such as leuco dyes, tetrazolium salts or shifted dyes. These dyes can be metal complexed or metal 45 complexable. Representative patents describing such dyes are U.S. Pat. Nos. 3,880,568; 3,931,144; 3,932,380; 3,932,381; and 3,942,987. Structures of illustrative dyes that can be blocked as described are as follows:



-continued



F. PUG's that form developing agents: Developing agents released can be color developing agents, black-and-white developing agents and cross-oxidizing developing agents. They include aminophenols, phenylenediamines, hydroquinones and pyrazolidones. Representative patents describing such developing agents are U.S. Pat. Nos. 2,193,015; 2,108,243; 2,592,364; 3,656,950; 3,658,525; 2,751,297; 2,289,367; 2,772,282; 2,743,279; 2,753,256; and 2,304,953.

Structures of preferred developing agents are:



where  $R_{5a}$  is hydrogen or alkyl of 1 to 4 carbon atoms and  $R_5$  is hydrogen or one or more halogen (e.g. chloro, bromo) or alkyl of 1 to 4 carbon atoms (e.g. methyl, ethyl, butyl) groups and alkoxy.



where  $R_s$  is as defined above.





where  $R_6$  is hydrogen or one or more alkyl, alkoxy or alkenedioxy groups of 1 to 4 carbon atoms and  $R_7$ ,  $R_8$ ,  $R_9$ ,  $R_{10}$  and  $R_{11}$  are individually hydrogen, alkyl of 1 to 4 carbon atoms (e.g. methyl, ethyl) lower hydroxyalkyl of 1 to 4 carbon atoms (e.g. hydroxymethyl, hydroxyethyl) or lower sulfoalkyl.

G. PUG's that are bleach inhibitors: Representative bleach inhibitors that can be blocked as described include the illustrative bleach inhibitors described in, for example, U.S. Pat. Nos. 3,705,801; 3,715,208 and German OLS No. 2,405,279. Structures of illustrative bleach inhibitors are:



wherein  $W_1$  is hydrogen, alkyl, such as ethyl and butyl, alkoxy, such as ethoxy and butoxy, or alkylthio, such as ethylthio and butylthio, for example containing 1 to 6 carbon atoms, and which may be unsubstituted or substituted;  $W_2$  is hydrogen, alkyl or aryl, such as phenyl;  $W_3$  and  $W_4$  are individually alkyl, such as alkyl containing 1 to 6 carbon atoms, for example ethyl and butyl or together can form a ring, such as morpholino;  $z$  is 1 to 6.

Other PUG's as described in the photographic art can also be blocked with a blocking group as described.

50 The blocked photographically useful compounds as described can be used in photographic materials and in ways that blocked photographic compounds have been used in the photographic art.

For example, the blocked photographic couplers can 55 be incorporated in photographic elements and/or photographic processing compositions, such that upon development in the presence of a dinucleophile reagent the exposed photographic element and coupler will be in reactive association with oxidized color developing 60 agent. When incorporated in a photographic element, the coupler compounds should as a rule be non-diffusible, that is they should be of such molecular size and configuration that they will not significantly diffuse or wander from the layer in which they are coated.

65 Photographic elements of the invention can be processed by conventional techniques in which color forming couplers and color developing agents are incorporated in separate processing solutions or compositions

or in the photographic element. Optionally, blocked color developing agents can be incorporated in the photographic element and simplified processing solutions used for processing the element.

The photographic elements can be single color elements or multicolor elements. Multicolor elements contain dye image-forming units sensitive to each of the three primary regions of the visible spectrum. Each unit can be comprised of a single emulsion layer or of multiple emulsion layers sensitive to a given region of the spectrum. The layers of the element, including the layers of the image-forming units, can be arranged in various orders as known in the photographic art. In an alternative format, the emulsions sensitive to each of the three primary regions of the spectrum can be disposed as a single segmented layer, such as by the use of microvessels as described in U.S. Pat. No. 4,362,806.

A typical multicolor photographic element comprises a support bearing a cyan dye image-forming unit comprising at least one red-sensitive silver halide emulsion layer having associated therewith at least one cyan dye-forming coupler, a magenta dye image-forming unit comprising at least one green-sensitive silver halide emulsion layer having associated therewith at least one magenta dye-forming coupler, and a yellow dye image-forming unit comprising at least one yellow dye-forming coupler. The element can contain added layers, such as filter layers, interlayers, overcoat layers, subbing layers, and the like.

The blocked photographically useful compounds as described can be present in and/or associated with one or more of the layers of the photographic element. The compounds can be in an emulsion layer and/or in an adjacent layer.

In the following discussion of materials useful in the emulsions and elements of the invention, reference will be made to Research Disclosure, December 1978, Item No. 17643, published by Industrial Opportunities Ltd., Homewell Havant, Hampshire, P09 1EF, U.K., the disclosures of which are incorporated herein by reference. The publication will be identified hereinafter by the term "Research Disclosure".

The silver halide emulsions employed in the elements can be comprised of silver bromide, silver chloride, silver iodide, silver chlorobromide, silver chloroiodide, 45 silver bromoiodide, silver chlorobromoiodide or mixtures thereof. The emulsions can include coarse, medium or fine silver halide grains. High aspect ratio tabular grain emulsions are specifically contemplated, such as those described by Wilgus U.S. Pat. Nos. 4,434,226, 50 Daubendiek et al 4,414,310, Wey 4,399,215, Solberg et al 4,433,048, Mignot 4,386,156, Evans et al 4,504,570, Maskasky 4,400,463, Wey et al 4,414,306, Maskasky 4,435,501 and 4,643,966 and Daubendiek et al 4,672,027 and 4,693,964. Also specifically contemplated are those 55 silver bromoiodide grains with a higher molar proportion of iodide in the core of the grain than in the periphery of the grain, such as those described in GB No. 1,027,146; JA No. 54/48,521; U.S. Pat. Nos. 4,379,837; 4,444,877; 4,665,012; 4,686,178; 4,565,778; 4,728,602; 60 4,668,614; 4,636,461; EP No. 264,954. The silver halide emulsions can be either monodisperse or polydisperse as precipitated. The grain size distribution of the emulsions can be controlled by silver halide grain separation techniques or by blending silver halide emulsions of differing grain sizes.

Sensitizing compounds, such as compounds of copper, thallium, lead, bismuth, cadmium and Group VIII

noble metals, can be present during precipitation of the silver halide emulsion.

The emulsions can be surface-sensitive emulsions, that is, emulsions that form latent images primarily on the surfaces of the silver halide grains, or internal latent image-forming emulsions, that is, emulsions that form latent images predominantly in the interior of the silver halide grains. The emulsions can be negative-working emulsions, such as surface-sensitive emulsions or unfogged internal latent image-forming emulsions, or direct-positive emulsions of the unfogged, internal latent image-forming type, which are positive-working when development is conducted with uniform light exposure or in the presence of a nucleating agent.

The silver halide emulsions can be surface sensitized. Noble metal (e.g., gold), middle chalcogen (e.g., sulfur, selenium, or tellurium), and reduction sensitizers, employed individually or in combination, are specifically contemplated. Typical chemical sensitizers are listed in *Research Disclosure*, Item 17643, cited above, Section III.

The silver halide emulsions can be spectrally sensitized with dyes from a variety of classes, including the polymethine dye class, which includes the cyanines, merocyanines, complex cyanines and merocyanines (i.e., tri-, tetra-, and poly-nuclear cyanines and merocyanines), oxonols, hemioxonols, styryls, merostryryls, and streptocyanines. Illustrative spectral sensitizing dyes are disclosed in *Research Disclosure*, Item 17643, cited above, Section IV.

Suitable vehicles for the emulsion layers and other layers of elements of this invention are described in *Research Disclosure* Item 17643, Section IX and the publications cited therein.

In addition to the couplers described herein the elements of this invention can include additional couplers as described in *Research Disclosure* Section VII, paragraphs D, E, F and G and the publications cited therein. These additional couplers can be incorporated as described in *Research Disclosure* Section VII, paragraph C and the publications cited therein.

The photographic elements of this invention can contain brighteners (*Research Disclosure* Section V), antifoggants and stabilizers (*Research Disclosure* Section VI), antistain agents and image dye stabilizers (*Research Disclosure* Section VII, paragraphs I and J), light absorbing and scattering materials (*Research Disclosure* Section VIII), hardeners (*Research Disclosure* Section X), coating aids (*Research Disclosure* Section XI), plasticizers and lubricants (*Research Disclosure* Section XII), antistatic agents (*Research Disclosure* Section XIII), matting agents (*Research Disclosure* Section XVI) and development modifiers (*Research Disclosure* Section XXI).

The photographic elements can be coated on a variety of supports as described in *Research Disclosure* Section XVII and the references described therein.

Photographic elements can be exposed to actinic radiation, typically in the visible region of the spectrum, to form a latent image as described in *Research Disclosure* Section XVIII and then processed to form a visible dye image as described in *Research Disclosure* Section XIX. Processing to form a visible dye image includes the step of contacting the element with a color developing agent to reduce developable silver halide and oxidize the color developing agent. Oxidized color developing agent in turn reacts with the coupler to yield a dye.

Preferred color developing agents are p-phenylene diamines. Especially preferred are 4-amino-3-methyl-N,N-diethylaniline hydrochloride, 4-amino-3-methyl-N-ethyl-N- $\beta$ -(methanesulfonamido)ethylaniline sulfate hydrate, 4-amino-3-methyl-N-ethyl-N- $\beta$ -hydroxyethylaniline sulfate, 4-amino-3- $\beta$ -(methanesulfonamido)ethyl-N,N-diethylaniline hydrochloride and 4-amino-N-ethyl-N-(2-methoxyethyl)-m-toluidine di-p-toluene sulfonic acid.

With negative-working silver halide, the processing step described above provides a negative image. The described elements are preferably processed in the known C-41 color process as described in, for example, the British Journal of Photography Annual of 1988, pages 196-198. To provide a positive (or reversal) image, the color development step can be preceded by development with a non-chromogenic developing agent to develop exposed silver halide, but not form dye, and then uniformly fogging the element to render unexposed silver halide developable. Alternatively, a direct positive emulsion can be employed to obtain a positive image.

Development is followed by the conventional steps of bleaching, fixing, or bleach-fixing, to remove silver or silver halide, washing, and drying.

In processing it is necessary that the described dinucleophile reagent, such as a hydroxylamine, be present in the processing solution that is to be used to release or unblock the blocked photographically useful compound at the time desired. The concentration of the dinucleophile reagent in the processing solution can vary depending on such factors as the particular processing solution components, the particular dinucleophile reagent, the processing time and temperature, the particular photographic element to be processed, the desired image and the like. When the dinucleophile reagent is present in a color developer solution, the concentration of the dinucleophile reagent is typically within the range of  $10^{-5}$  moles to 1 mole per liter of solution.

The blocked photographically useful compounds according to the invention can be prepared by methods and steps known in the organic compound synthesis art.

A typical method of preparing a blocked photographically useful compound is as follows:

### SYNTHESIS I

#### A. Preparation of an intermediate 2,2-dimethyl-3-oxobutyryl chloride (G1)



This illustrative intermediate compound G1 can be reacted with a photographically useful group (PUG) to provide a blocked photographically useful compound as described.

A 2-liter, 3-necked round-bottomed flask containing ethyl acetoacetate (65 g, 0.5 mole), t-butanol (200 ml), and tetrahydrofuran (200 ml) was fitted with thermometer, mechanical stirrer, nitrogen inlet, and addition funnel topped with an ice water condenser. The mixture was cooled to 0° C. and stirred vigorously under a slow nitrogen stream while adding potassium t-butoxide (56 g, 0.5 mole) slowly (temp. <20° C.). A homogeneous solution resulted after about 5 minutes. Methyl iodide (32 ml, 0.5 mole) was added via the addition funnel while the temperature rose to about 10° C. The ice bath was replaced with a water bath at room temperature (20° C.) before stirring the mixture for an additional 30 minutes while potassium iodide precipitated. The mixture was cooled again to 0° C. before adding more methyl iodide (40 ml) and then potassium t-butoxide (56 g, 0.5 mole) (temp. <30° C.). The mixture was stirred at room temperature for 48 hours and then diluted with about 1 liter of water and 0.5 liter of saturated NaCl solution before the mixture was extracted with ether. The ether solution was washed with 0.1N NaOH and then with 1N HCl, dried over magnesium sulfate, and concentrated to an oil. The crude dimethylated ethyl acetoacetate (64 g, 81% yield) had an nmr spectrum that was consistent with the expected compound.

The crude dimethylated ester (64 g, approx. 0.4 mole), NaOH (48 g, 1.2 mole), water (320 ml), and a trace of indicator dye (Metanil Yellow) were stirred for 18 hours until a homogeneous solution resulted. Residual alkali-insoluble material was removed by washing with a small amount of ether. The alkaline solution was then cooled in ice water and neutralized carefully with concentrated HCl (approx. 100 ml) until the indicator dye turned purple. Saturated NaCl was added to the cold solution before extracting several times with methylene chloride. The extracts were dried over sodium sulfate, filtered and concentrated at 30° C. to yield the crude acid as an oil (50 g) (the acid solidifies at ice temperatures). The nmr spectrum showed that a small amount of ethanol was present in the crude acid. In order to avoid excessive decarboxylation, the acid was used immediately by reacting with oxalyl chloride (75 ml, 0.86 mole) and a trace of triethylamine at room temperature for 24 hours. The mixture was concentrated at 30° C. using a rotary evaporator with water aspirator vacuum. Excess oxalyl chloride was removed by codistillation with methylene chloride to yield crude 2,2-dimethyl-3-oxobutyryl chloride (49 g, 82%). A portion of the crude (45 g) was distilled through a six inch Vigreux column under water aspirator vacuum (bp 50°-55° C.) to yield purified colorless product (30 g, 67%). A small amount of impurity containing an ethoxy group distilled with the later fractions of product. This impurity could be avoided by complete removal of ethanol prior to acid chloride formation.

Other illustrative intermediate compounds can be prepared in a similar manner. Illustrative compounds include G2 and G3 and are represented by the formulas:



-continued

The following is a specific illustrative synthesis of a blocked filter dye involving reaction with compound G2:  
10

## SYNTHESIS EXAMPLE A

## Preparation of Compound (I)



(B)



(C)

(D)



(E)

(F)

-continued



DMAP herein is 4-dimethylaminopyridine. DBU herein is 1,8-diazabicyclo[5.4.0]undec-7-ene. Ether means ethyl ether. EtiPr<sub>2</sub>N herein means ethyldiisopropylamine. Me herein means CH<sub>3</sub>—. Et herein means C<sub>2</sub>H<sub>5</sub>. Temperatures herein are ° C. unless otherwise indicated.

### Preparation of (A)

Ethyl bromide (500 g, 4.6 mole), o-anisidine (370 g, 3.0 mole), and isopropanol (1 l) were refluxed for 16 hours. The hot solution was poured into a container and cooled with ice. The crystalline hydrobromide salt was filtered, washed with cold isopropanol and ether. Recrystallization from a minimum volume of hot isopropanol with cooling at 0° overnight yielded 402 g (58%) of 35 (A).

### Preparation of (B)

Water (400 ml), conc. HCl (80 ml), and p-aminobenzoic acid (31.4 g, 0.21 mole) were mixed. After cooling the mixture to 0°, ice (100 g) and sodium nitrite (14.3 g, 0.21 mole) were added. After a few minutes when all of the nitrite had dissolved, a solution of (A) (48.0 g, 0.21 mole) in aqueous HCl (40 ml of conc. HCl, 200 ml of H<sub>2</sub>O) was slowly added while maintaining the temperature near 0°. Sodium acetate (140 g) was slowly added to promote coupling. After stirring about 30 minutes, the mixture was filtered to obtain a mixture of dye and triazene. The triazene was rearranged to dye by stirring the crude product with acetic acid (about 200 ml) for 2 days at room temperature (20°) (or by heating for about 2 hours at 50°). The dye which precipitated from the acetic acid was filtered off and washed with methanol to yield 41.7 g (67%) of (B).

### Preparation of (C)

The acidic dye (B) (41.7 g, 0.14 mole) was esterified by heating with dodecyliodide (45.6 g, 0.15 mole), ethyldiisopropylamine (19.4 g, 0.15 mole), and DMF (200 ml) at 100° for 3 hours. The crude mixture was 60 diluted with ether, washed with 0.05N HCl and water, dried over MgSO<sub>4</sub>, concentrated to an oil, and crystallized from methanol to yield 44.5 g (68%) of ballasted dye (C).

### Preparation of (D)

Ballasted dye (D) (12.3 g, 0.0264 mole) and 2,6-lutidine (3.2 g, 0.03 mole) were dissolved in dichlorometh-

ane (200 ml) cooled to about 15°. Phosgene (30 ml of 1M solution in toluene, 0.03 mole) was added slowly before stirring the mixture for 20 minutes. The mixture was washed with cold aqueous 0.05N HCl and ice water before drying over  $MgSO_4$ . Crude carbamyl chloride (D) was obtained by concentration in vacuo. This was used directly in the reaction to form (I) without further purification.

### Preparation of (E)

Commercially available 3-nitro-4-hydroxybenzyl alcohol (16.9 g, 0.1 mole) was hydrogenated at (40 psi) (3 atm) 280 Kilo Pascals in dioxane (300 ml) using 1 g of 5% Pd on carbon as catalyst. After the catalyst was filtered off, the solution was concentrated to form (E) as a crystalline solid (10 g, 72%).

### Preparation of (F)

Aminophenol (E) (2.78 g, 0.02 mole) and 2,6-lutidine (2.36 g, 0.022 mole) were mixed with p-dioxane (40 ml). Methanesulfonic anhydride (3.48 g, 0.02 mole) was then added. After  $\frac{1}{2}$  hour, the mixture was diluted with ethyl acetate and washed twice with salt water (100 ml of saturated NaCl plus 15 ml of 1N HCl). After drying over MgSO<sub>4</sub>, the ethyl acetate extract was concentrated to a solid residue. Crystallization from ethyl acetate-heptane yielded 3.2 g (75%) of product (F).

### Preparation of (H)

A homogeneous solution of triethylamine (11.2 ml, 0.08 mole) and phenolic compound (F) (10.9 g, 0.05 mole) in tetrahydrofuran (100 ml) was cooled to  $-20^{\circ}$  under a nitrogen atmosphere. A solution of acid chloride (G2) (8.75 g, 0.05 mole) in methylene chloride (50 ml) was then added. The mixture was warmed to room temperature for a few minutes, diluted with more solvent, and washed with 0.1N HCl. The organic layer was dried with magnesium sulfate and concentrated to an oil (19 g) which contained a small amount of solvent but was pure enough for use in the next step.

### Preparation of (I)

65 Dye carbamyl chloride (D) (8.0 g, 0.015 mole), hydroxy compound (H) (5.3 g, 0.015 mole), DMAP (3.7 g, 0.03 mole), and DBU (6.8 g, 0.045 mole) were stirred in methylene chloride (30 ml) solution at room tempera-

ture for 30 minutes. The reaction was quenched by washing with aqueous 0.5N HCl, and the organic layer was dried over magnesium sulfate, and concentrated to a crude oil. The crude product was chromatographed on 750 g of silica gel using ethyl acetate:heptane (1:3) as eluent. Purified shifted filter dye (I) (7 g, 55%) was obtained as a glassy solid.

Another illustrative synthesis of a blocked photographically useful compound is as follows:

### SYNTHESIS II



(J)



(L)

With stirring, 27.5 g. of compound J was dissolved in a solution of 50 ml of triethylamine and 450 ml of pyridine. Compound K (25.0 g) was added dropwise over a period of five minutes. The resulting mixture was stirred overnight at room temperature, concentrated under vacuum, and the residue stirred with 500 ml of ethyl ether. The mixture was filtered. The filtrate was washed five times with 500 ml portions of water and then with saturated aqueous sodium chloride solution. The resulting organic layer was dried over anhydrous magnesium sulfate. The solution was filtered and concentrated to provide 30 grams of light gold oil. Upon standing the light gold oil solidified. The solid was broken up by stirring with petroleum ether (bp 30°-60°) and then collected by filtration to provide 22.5 g of white solid melting at 74°-75° C. The desired compound was identified by NMR.

H NMR (CDCl<sub>3</sub>) 7.2-7.3 (triplet, 2H); 6.9-7.0 (doublet, 2H); 6.8-6.9 (triplet, 1H); 3.6 (singlet, 2H); 2.5-2.6 (multiplet, 3H); 2.0-2.1 (multiplet, 1H); 1.5-1.9 (multiplet, 4H); 1.4-1.5 (singlet, 3H); and 1.2-1.3 ppm (singlet, 6H).

<sup>13</sup>C NMR (CDCl<sub>3</sub>) 206.6, 170.0, 158.5, 146.5, 128.6, 119.2, 112.8, 63.8, 57.1, 44.4, 39.9, 37.4, 27.0, 23.3, 21.8, and 20.7 ppm.

In chemical systems that require a blocked reagent, 10 the reagent can be released by reaction with a dinucleophile reagent. The reagent can be released by any dinucleophile reagent that is compatible with the particular chemical system. Selection of an optimum dinucleophile reagent and a particular blocked reagent will depend upon the particular chemical system, the desired 15 end use of the blocked reagent, the particular conditions used for release. The blocking group can be as described in such blocked reagents.

The following examples further illustrate the invention.: 20

### EXAMPLE 1

Model studies were conducted on esters E-1 through E-5 to determine the possible rate enhancement which 25 could be attained by using a dinucleophile rather than a mononucleophile to promote the removal from a phenolic moiety of a blocking group of this invention. Aqueous solutions A, B, and C, each containing 50% by volume of acetonitrile were prepared as follows (a separate solution A for each ester):

|             |                                                                         |
|-------------|-------------------------------------------------------------------------|
| Solution A: | $2.5 \times 10^{-4}$ M ester (or $2.5 \times 10^{-5}$ M E-1); 0.2 N KCl |
| Solution B: | 25% by volume carbonate buffer (ionic strength 0.75); 0.05 N KCl        |
| Solution C: | Solution B with added 0.05 M hydroxylamine                              |

Then equal volumes of A and B (or A and C) were 40 mixed at 25° C. to give a pH 10.0 solution and the reaction was followed by spectrophotometric measurements of the phenol (272 nm) or p-nitrophenol (402 nm) produced with time. In each case a reaction half-life ( $t_{1/2}$ ) was calculated from the equation  $t_{1/2} = \ln(2)/k$ , where 45  $\ln(2)$  is the natural logarithm of 2 and k is the pseudo first-order rate constant calculated for the reaction. Smaller half-lives thus indicate more rapid reactions. The A+B combination provides an alkaline solution in 50 which the main reactant is hydroxide ion (a mononucleophile) while in the A+C combination the active reactant is hydroxylamine (a dinucleophile). A ratio of the A+B half-life to the A+C half-life provides a measure of rate enhancement due to participation of hydroxylamine in the deblocking reaction. The results are shown in Table I:

TABLE I

|                 | $t_{1/2} A + B$  | $t_{1/2} A + C$ | Ratio            |
|-----------------|------------------|-----------------|------------------|
| E-1 (Invention) | $62 \times 10^3$ | 1.7             | $36 \times 10^3$ |

TABLE I-continued

|                                                                                   | $t_{1/2}A + B$    | $t_{1/2}A + C$ | Ratio             |
|-----------------------------------------------------------------------------------|-------------------|----------------|-------------------|
|  | $800 \times 10^3$ | 8.6            | $93 \times 10^3$  |
| E-2 (Invention)                                                                   |                   |                |                   |
|  | $20 \times 10^6$  | 6.3            | $3.2 \times 10^6$ |
| E-3 (Invention)                                                                   |                   |                |                   |
|  | $9.3 \times 10^3$ | 200            | 47                |
| E-4 (Comparison)                                                                  |                   |                |                   |
|  | $130 \times 10^3$ | 785            | 166               |
| E-5 (Comparison)                                                                  |                   |                |                   |

It can be seen from Table I that the rate enhancement due to dinucleophile (hydroxylamine) participation in the hydrolysis of esters E-1, E-2, and E-3 using blocking groups of the invention are twenty to seventy thousand times greater than for the comparison blocking groups in esters E-4 and E-5. The esters representing blocking groups of the invention give the rapid deblocking of a few seconds needed for pH 10 processing while maintaining excellent resistance toward base hydrolysis. These results would predict that a blocked PUG according to the invention would be quite stable under pre-processing storage conditions since only mononucleophiles are present in storage yet capable of rapid PUG release at a desired time during processing.

#### EXAMPLE 2

This example demonstrates that a blocked electron transfer agent (ETA) when incorporated in a photographic light sensitive element can be deblocked rapidly when the processing solution contains the dinucleophile hydroxylamine sulfate (HAS). A green sensitized silver bromoiodide gelatin emulsion (0.7 micron grain size) was mixed with a coupler dispersion comprising cyan coupler C-1 dispersed in half its weight of di-n-butyl phthalate and a blocked ETA compound of the invention dispersed in twice its weight of N,N-diethyl lauramide. The resulting mixture was coated on a photographic film support according to the following format (amounts of each component are given in mg/m<sup>2</sup> with silver halide counted as silver):

|                 |                                                                                                                                          |
|-----------------|------------------------------------------------------------------------------------------------------------------------------------------|
| OVERCOAT LAYER: | Gelatin (5382); bis(vinylsulfonyl-methyl) ether hardener (2% of total gelatin weight)                                                    |
| EMULSION LAYER: | Gelatin (3229); green-sensitized AgBrI emulsion (877); cyan coupler C-1 (969); and a blocked ETA compound (levels indicated in Table II) |
| FILM SUPPORT:   |                                                                                                                                          |

-continued

#### Cyan Coupler C-1:



#### Blocked ETA Compound 1:



#### Blocked ETA Compound 2:



Each photographic element was imagewise exposed to light through a graduated density test object in a

commercial sensitometer to provide a developable latent image (3000° K. light source, 0-4 step wedge, with

3 of the invention and comparison Compound 3U of the corresponding unblocked structures:



Wratten 99 plus 0.5ND filter. Wratten is a trademark). The resulting photographic film was then developed and processed in a commercial C-41 development process of Eastman Kodak Company, U.S.A. without the final stabilizer step. This process and the processing compositions for the process are described in, for example, British Journal of Photography Annual 1988, Pages 191-199. The development process was carried out with and without hydroxylamine sulfate (HAS) in the color developer solution. 30 35

Densitometric measurements made with red light are shown in Table II wherein the values in parentheses are for the samples processed in the developer without HAS.  $D_{min}$  is the average fog level. Gamma is the maximum contrast between two density points which are  $0.4 \log E$  apart, taken as the difference from the gamma of the control sample which contains no blocked ETA compound. Photographic speed is also taken relative to the control sample (set at 100) and is measured at 0.15 density above fog.

30 mat on a poly(ethylene terephthalate) film support (unless otherwise specified, component amounts are given in mg/m<sup>2</sup> with silver halide counted as silver):

|                    |                                                                                                                       |
|--------------------|-----------------------------------------------------------------------------------------------------------------------|
| OVERCOAT<br>LAYER: | Gelatin (2691); bis(vinylsulfonyl-methyl) ether hardener (1.75% of total gelatin weight)                              |
| EMULSION<br>LAYER: | Gelatin (3767); unsensitized AgBr emulsion (906); masking coupler indicated in Table III (1.08 mmole/m <sup>2</sup> ) |
| FILM SUPPORT:      |                                                                                                                       |

Unexposed strips of this coated element were soaked 1 minute in a fixing solution to remove silver halide, washed, and then immersed in one of the following processing solutions at temperatures conventionally used for processing in a KODAK C-41 process:

TABLE II

| Blocked<br>ETA | Amt. Added<br>(mmole/m <sup>2</sup> ) | Dmin        | Relative<br>Gamma Difference |         | Relative Speed |
|----------------|---------------------------------------|-------------|------------------------------|---------|----------------|
| None           | —                                     | 0.08 (0.07) | 0                            | (0)     | 100 (100)      |
| Compd. 1       | 0.215                                 | 0.07 (0.06) | -0.01                        | (-0.06) | 102 (100)      |
| "              | 0.431                                 | 0.07 (0.06) | -0.08                        | (-0.09) | 103 (101)      |
| "              | 1.076                                 | 0.07 (0.05) | -0.54                        | (-0.35) | 105 (100)      |
| Compd. 2       | 0.215                                 | 0.09 (0.06) | +0.10                        | (-0.02) | 108 (100)      |
| "              | 0.431                                 | 0.09 (0.06) | -0.04                        | (-0.01) | 109 (100)      |
| "              | 1.076                                 | 0.09 (0.06) | -0.53                        | (-0.18) | 109 (101)      |

The data in Table II show that the compounds of the 60 invention deblock rapidly in the presence of hydroxylamine sulfate to release an ETA compound which can produce a significant speed increase even at low addenda levels.

### EXAMPLE 3

To demonstrate the use of a shifted masking coupler, photographic elements were prepared using Compound

P-1: pH 10 carbonate buffer  
P-2: pH 10 carbonate buffer with 0.024M hydroxylam-

P-3: C-41 color developer with hydroxylamine sulfate

1-5. C. VI color developer with hydroxylamine sulfate omitted

## P-4: C-41 color developer solution containing hydroxylamine sulfate

The results are presented in Table III:

TABLE III

| Treatment       | Density at 520 nm |          |
|-----------------|-------------------|----------|
|                 | Compd. 3U         | Compd. 3 |
| Fixed Only      | 1.25              | 0.02     |
| P-1: 10 Minutes | 1.25              | 0.02     |
| P-2: 10 Minutes | 1.25              | 1.10     |
| P-3: 10 Minutes | 1.25              | 0.02     |
| P-4: 1 Minute   | 1.25              | 0.50     |
| P-4: 10 Minutes | 1.25              | 1.25     |

The data in Table III demonstrate that the blocked masking coupler Compound 3 of the invention is not unblocked by extended treatment with an alkaline bath (P-1) containing carbonate and hydroxide ions or a developer solution (P-3) which does not contain a dinucleophile. However, when the dinucleophile hydroxylamine is added to either of these solutions, as in P-2 and P-4, the blocking group is readily removed from the blocked masking coupler Compound 3 to form the corresponding unblocked Compound 3U. The absorption maximum of blocked Compound 3 is shifted to about 375 nm so that it absorbs very little green light until it is

dispersed in half its weight of di-n-butyl phthalate. These were then coated in the following format (unless otherwise specified, component amounts are given in mg/m<sup>2</sup> with silver halide counted as silver):

|   |                 |                                                                                                                                                      |
|---|-----------------|------------------------------------------------------------------------------------------------------------------------------------------------------|
| 5 | OVERCOAT LAYER: | Gelatin (2691); bis(vinylsulfonylmethyl) ether hardener (1.75% of total gelatin weight)                                                              |
|   | EMULSION LAYER: | Gelatin (3767); unsensitized AgBrI emulsion (1615); cyan image coupler C-1 (754); masking coupler indicated in Table V (0.108 mmole/m <sup>2</sup> ) |
|   | FILM SUPPORT:   | with antihalation backing                                                                                                                            |

10 Film strips of the above coatings were step-exposed through a Wratten 12 (minus blue) filter, processed (C-41) as in Example 2, and the photographic parameters measured as presented in Table V (density to green light was measured for unexposed fixed strips and for low and high exposure areas of processed strips; photographic speed of the red image is relative to the control at 100):

TABLE V

| Added Masking Coupler | Green Density @ Exp. |      |      | Red Image |       |      |
|-----------------------|----------------------|------|------|-----------|-------|------|
|                       | None                 | Low  | High | Dmax      | Gamma | Spd. |
| Control               | None                 | 0.06 | 0.06 | 0.38      | 2.44  | 2.33 |
| Comparison            | Compd. 3U            | 0.21 | 0.24 | 0.40      | 2.59  | 2.24 |
| Invention             | Compd. 3             | 0.08 | 0.26 | 0.43      | 2.62  | 2.42 |

unblocked by a dinucleophile during processing.

#### EXAMPLE 4

Strips of the same coated photographic elements described above in Example 3 were either fixed to remove silver halide or were given a stepped exposure to white light and then C-41 processing as in Example 2. Densities to red, green, and blue light for low and high exposure steps were measured as shown in Table IV:

TABLE IV

| Compd.       | Exposure     |               |             |              |               |             |
|--------------|--------------|---------------|-------------|--------------|---------------|-------------|
|              | Blue Density | Green Density | Red Density | Blue Density | Green Density | Red Density |
| 3U           | 3            | 3U            | 3           | 3U           | 3             | 3           |
| None (Fixed) | 0.64         | 0.85          | 1.18        | 0.08         | 0.09          | 0.04        |
| Low          | 0.65         | 0.71          | 1.22        | 0.90         | 0.13          | 0.11        |
| High         | 0.24         | 0.16          | 0.36        | 0.24         | 1.82          | 2.08        |

The Table IV data for coatings containing high levels of masking coupler (and none of the normally present image coupler) demonstrate that a positive masking image to blue and green light is produced in addition to the negative image to red light. The no-exposure sample containing blocked masking coupler Compound 3, however, shows the added advantage of extremely low density to green light compared to the counterpart Compound 3U in which the same chromophore is unblocked. Before processing the blocked masking coupler allows more green light to pass to lower photographic layers and yet after processing it can provide the desired compensation for unwanted spectral absorptions of the image dye.

#### EXAMPLE 5

This example demonstrates the use of a blocked masking coupler in the presence of a main image coupler in a monochrome layer. Dispersions were made as in Example 3 but with added cyan coupler C-1 dis-

35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865

-continued



5

Strips of each coating were soaked at 38° C. in C-41 developer or in the same C-41 developer formulation from which hydroxylamine sulfate (HAS) had been omitted. The rate of deblocking of each filter dye was followed by measuring the density at the absorption maximum of the unblocked dye at selected time intervals. The results are presented in Table VI:

TABLE VI

| Cmpd. | λ <sub>max</sub><br>(Un-blocked) | Filter Dyes:                                 |      |      |                               |      |      |
|-------|----------------------------------|----------------------------------------------|------|------|-------------------------------|------|------|
|       |                                  | Density at λ <sub>max</sub> of Unblocked Dye |      |      |                               |      |      |
|       |                                  | (Comparative Example)<br>C-41 Dev. (No HAS)  |      |      | (Invention)<br>C-41 Developer |      |      |
| Cmpd. | λ <sub>max</sub><br>(Un-blocked) | 0'                                           | 1'   | 10'  | 0'                            | 1'   | 10'  |
| 4     | 440 nm                           | 0.05                                         | 0.09 | 0.10 | 0.05                          | 1.08 | 1.10 |
| 5     | 440 nm                           | 0.03                                         | 0.03 | 0.05 | 0.03                          | 0.08 | 0.71 |

10

15

20

25

TABLE VI-continued

| Cmpd. | λ <sub>max</sub><br>(Un-blocked) | Filter Dyes:                                 |      |      |                               |      |      |
|-------|----------------------------------|----------------------------------------------|------|------|-------------------------------|------|------|
|       |                                  | Density at λ <sub>max</sub> of Unblocked Dye |      |      |                               |      |      |
|       |                                  | (Comparative Example)<br>C-41 Dev. (No HAS)  |      |      | (Invention)<br>C-41 Developer |      |      |
| 6     | 495 nm                           | 0.03                                         | 0.05 | 0.06 | 0.05                          | 0.84 | 0.89 |

It can be seen from the densities at the processing times shown in Table VI that the blocked filter dyes of this invention are released much too slowly in the absence of hydroxylamine to be useful in pH 10 photographic processes. The blocked filter dyes have the desirable stability for long-term keeping at the pH 5.5-6 in an unprocessed coating. In accelerated keeping tests at least 95% of the blocked filter dye was recovered unchanged. However, in the commercial C-41 developer, which contains the hydroxylamine dinucleophile, useful filter dye densities are achieved quite rapidly.

## EXAMPLES 7-33

The following blocked photographically useful compounds can be prepared by the methods described. These blocked compounds can be incorporated and processed in a photographic element as described, such as in the element and process of Example 1: (The example number is given for each compound.)

## Image Couplers:



7.

-continued

8.



9.



10.



-continued





-continued

14.



15.

#### Development Accelerators and Electron Transfer Agents:



16.



17.



18.



19.

35

5,019,492

-continued



36

20.



21.



22.



23.



24.



25.

Dox Scavenger:Color Developers:

26.



27.

Antifoggants:

-continued



28.

Other Compounds:

-continued

33.



34.



35.



36.



The invention has been described in detail with particular reference to particular embodiments thereof, but it will be understood that variations and modifications can be effected within the spirit and scope of the invention.

What is claimed is:

1. A photographic element comprising a support bearing at least one silver halide photographic emulsion layer and a blocked photographically useful compound comprising a photographically useful group and a

blocking group that is capable of releasing the photographically useful group upon processing the photographic element wherein the blocking group

- 65 (a) comprises two electrophilic groups, the least electrophilic of which is bonded directly or through a releasable timing group to the photographically useful group;
- (b) is capable of reacting with a dinucleophile; and,

(c) the two electrophilic groups are separated from each other by a substituted atom that enables a nucleophilic displacement reaction to occur with release of PUG upon processing the photographic element in the presence of a dinucleophilic reagent.

2. A photographic element as in claim 1 wherein the blocked photographically useful compound is represented by the formula:



10

wherein

$E_1$  and  $E_2$  are independently electrophilic groups, wherein  $E_1$  is more electrophilic than  $E_2$ ;

$T_1$  and  $T_2$  are individually releasable timing groups;

$Y^1$  is a substituted atom that provides a distance between  $E_1$  and  $E_2$  that enables a nucleophilic displacement reaction to occur with release of PUG upon processing the photographic element in the presence of a dinucleophile;

PUG is a photographically useful group capable of being released upon processing the photographic element;

$x$  and  $y$  are independently 0 or 1; and,

$n$  is 1 or 2.

3. A photographic element as in claim 1 wherein the blocked photographically useful compound is represented by the formula:



25

wherein

$R_3$  is unsubstituted or substituted alkyl, unsubstituted or substituted aryl, or the atoms necessary with  $Z$  to complete a ring with  $Y^2$ ;

$Z$  represents the atoms necessary to complete a ring with  $R_3$  and  $Y^2$

$Y^2$  is a substituted carbon atom that provides a distance between the carbonyl groups that enables a

15

20

25

30

nucleophilic displacement reaction to occur with release of PUG upon processing the photographic element in the presence of a dinucleophile;  $q$  and  $z$  are independently 0 or 1;  $T_3$  is a releasable timing group; and, PUG is a photographically useful group.

4. A photographic element as in claim 1 wherein the blocked photographically useful compound is represented by the formula:



15

wherein  $R_4$  is unsubstituted or substituted alkyl or unsubstituted or substituted aryl; PUG is a photographically useful group;  $T_4$  is a releasable timing group; and,  $r$  is 0 or 1.

5. A photographic element as in claim 1 wherein the blocked photographically useful compound is represented by the formula:



20

25

wherein PUG is a photographically useful group;  $T_5$  is a releasable timing group; and  $s$  is 0 or 1.

6. A photographic element as in claim 1 wherein the PUG is a coupler, dye, nucleating agent, development accelerator, inhibitor releasing developer, color developer, development restrainer, antifoggant, bleach accelerator, bleach inhibitor, hardener, silver halide solvent, or precursors thereof.

7. A photographic element as in claim 1 wherein the blocked photographically useful compound is



-continued



wherein Q is hydrogen or a coupling-off group.

65

8. A process of forming a photographic image in an exposed photographic element as defined in claim 1 comprising developing said element with a photo-

graphic silver halide color developing agent in the presence of a dinucleophilic reagent.

\* \* \* \*